

# UNITED STATES PATENT OFFICE.

FRANK S. HODSON, OF PHILADELPHIA, PENNSYLVANIA.

## METALLIC ALLOY.

1,276,916.

Specification of Letters Patent. Patented Aug. 27, 1918.

No Drawing.

Application filed August 28, 1917. Serial No. 188,555.

To all whom it may concern:

Be it known that I, FRANK S. HODSON, a citizen of the United States, residing at Philadelphia, in the county of Philadelphia and State of Pennsylvania, have invented 5 certain new and useful Improvements in Metallic Alloys, of which the following is a specification.

My invention consists of an improved 10 metallic alloy. One object of my invention is to provide an improved metallic alloy of high tensile strength and hardness and which is particularly suitable for use in the manufacture of high tensile strength die 15 castings, drawn rods and bars, and sheets, etc.

According to my invention, my improved metallic alloy is composed of zinc, aluminum and copper.

20 In carrying out my invention, the quantities of the metals forming my improved alloy may vary preferably in the following relative proportions:—

25 Zinc----- 80% to 85%  
Aluminum----- 18% to 14%

the remaining percentage being completed with copper.

In specifying these metals it will, of 30 course, be understood that I contemplate employing them as commercially furnished, and that therefore the usual variations in the purity of each are ignored. For instance, in commercial zinc there is not infrequently present as high as five per cent. of lead. Such normal commercial impurities do not, however, injuriously affect the character of the resultant product in my experience, and their presence may be tolerated without departure from my invention.

40 In manufacturing the alloy I prefer to proceed as follows: The copper is first melted and the aluminum is then added thereto, thus forming what may be termed a mother-

alloy, to which the zinc is added. The zinc 45 may be added either to the aluminum copper alloy in its initial condition of melting or the mother-alloy may be first prepared and re-melted for addition of the proper proportion of zinc. As a definite example of 50 proportions with the several ingredients in a condition of relatively high purity I would state that the mother-alloy may be composed of eight per cent. of copper and ninety-two per cent. of aluminum, and the 55 ultimate alloy may consist of eighteen per cent. of this mother-alloy, and eighty-two per cent. of zinc.

In carrying out tests with the alloy it has been found that in sand castings the 60 tensile strength of the alloy approximates to 36,000 pounds to the square inch, and that under the Brinnel test the alloy shows a hardness of 35.

Having thus described my invention, what 65 I claim as new and desire to secure by Letters Patent is:

1. The herein described composition of matter, consisting of an alloy of copper, aluminum and zinc, the aluminum being present in large excess of the copper and the zinc being present in large excess of the aggregate amount of aluminum and copper together, substantially as described.

2. The herein described composition of 75 matter consisting of a metallic alloy in the following proportions, zinc eighty to eighty-five parts, aluminum eighteen to fourteen parts, and copper two to one parts, substantially as described.

In testimony whereof I have signed my name to this specification in the presence of two subscribing witnesses.

FRANK S. HODSON.

Witnesses:

CHAS. E. POTTS,  
MARY A. INGLAR.